

## UNITED STATES PATENT OFFICE

2,375,175

## SMOKELESS POWDER PROCESS

Charles Earnest Silk, Alton, Ill., assignor to Olin  
Industries, Inc., East Alton, Ill., a corporation  
of Delaware

No Drawing. Application January 1, 1944,  
Serial No. 516,716

17 Claims. (Cl. 52—22)

This invention relates to explosives and particularly to smokeless powder and provides an improved process of manufacturing spherical grains thereof. This application is a continuation in part of my prior copending application, Serial No. 333,107 filed May 3, 1940.

Spherical grains of propellant powder in accordance with U. S. Patent 2,027,114 have heretofore been manufactured by a procedure in which a lacquer, formed by dispersing a smokeless powder base in a suitable solvent, was distributed in the form of particles in a non-solvent medium, these particles being subsequently transformed to globules at atmospheric pressure and hardened, by progressively raising the temperature and vaporizing the solvent, to form the desired gelatinized grains.

An object of the present invention, generally stated, is to provide an improved process for the manufacture of spherical grains of propellant powder.

Another object of the invention is to provide a process for the manufacture of spherical grains of propellant powder wherein a smaller quantity of solvent is required than heretofore.

A further object of the invention is to provide a process whereby the formation of spherical grains of smokeless powder is facilitated and expedited.

Other objects will become apparent to those skilled in the art when the following description is read.

In accordance with the present invention, generally stated, the foregoing objects may be accomplished by distributing particles of a lacquer, formed by dispersing a smokeless powder base in a limited quantity of volatile solvent, in a suitable non-solvent medium, the quantity of solvent utilized being insufficient, at normal atmospheric temperature, to render the lacquer workable to the extent necessary. The present invention contemplates that the lacquer be rendered workably fluid by the combined action of solvent and heat, and particularly that the temperature of the mixture be elevated to a point at which the heat augments the action of the solvent in increasing the fluidity of the lacquer particles. In order to prevent neutralization of the heat effect by evaporation of the solvent, however, an important aspect of the present invention resides in the feature that the pressure on the mixture is increased to an extent sufficient to inhibit evaporation of the solvent at the temperatures encountered which are higher than the normal (atmospheric pressure) boiling point of the mix-

ture. While the lacquer is being rendered and maintained fluid by the combined action of solvent and heat (under pressure) the mixture is agitated, so as to cause the particles of lacquer

- 5 to assume a globular shape. When the particles of lacquer have assumed the desired shape, they are set in that shape by reducing the pressure on the mixture. The pressure reduction may be accomplished either by venting the sealed vessel 10 in which the mixture is being agitated while maintaining the heat (which results in evaporation of the solvent from the formed globules) or by lowering the temperature of the mixture (which results in "freezing" the formed globules). 15 By either of these methods reduction of pressure within the vessel to atmospheric may be accomplished; or the pressure reduction may be interrupted at an intermediate point dependent upon the degree of venting or the degree of chilling. 20 In any event, after the pressure has been reduced and the globules are set, the solvent is further removed from the globules, as by distillation.

In accordance with this procedure, therefore, 25 advantage is taken of the fact that a rise in temperature of a given solution of a smokeless powder base such as nitrocellulose in a suitable solvent will be accompanied by a marked decrease in viscosity. By carrying out the step of

- 30 shaping the grains at an elevated pressure it becomes possible to resort to higher temperatures and thus to reduce the amount of solvent required in the process and also to produce more perfectly shaped grains of improved uniformity 35 of granulation in a shorter time. In accordance with one embodiment of the invention, by lowering the temperature of the suspension after the particles of lacquer have become transformed into the desired globular shape, the particles become "frozen" in the acquired shape and the volatile solvent may be removed, as by evaporation, from the grains while in suspension without impairing their form. In accordance with another embodiment, the sealed treating vessel 40 is vented after the particles of lacquer have become transformed into the desired globular shape and the reduction of pressure incident to such venting causes the volatile solvent to be removed from the grains while in suspension. In either case, however, the solvent may be removed at a more rapid rate than heretofore, because the amount of solvent is less, and because, with the higher solids content of the globules and therefore the smaller amount of shrinkage thereof on 45 evaporation of solvent, grains of suitable shape 50 55

and density result even with rapid rates of evaporation of the solvent.

These advantages were not obtainable in the processes heretofore in use in the manufacture of spherical grains of propellant powder since the step of shaping the grains occurred at normal atmospheric pressure and at or slightly above normal atmospheric temperature and the temperature then raised to effect the removal of solvent by evaporation. Accordingly, larger amounts of solvent were required and a protracted and carefully controlled distillation period for the removal of solvent was necessary in order to secure grains of the desired shape and density.

The process of this invention may be applied in the manufacture of smooth-surfaced spherical grains of any suitable smokeless powder base. The base may, for example, consist of nitrocellulose of any desired degree of nitration, viscosity, or physical form or of a mixture of different types of nitrocellulose. The nitrocellulose may be replaced wholly or in part by other high molecular weight smokeless powder bases, such as nitrostarch, capable of being dispersed in a volatile solvent and of being converted to a coherent gelatinized solid on evaporation of the solvent. The smokeless powder base may also contain other active explosive ingredients such as nitro aromatic compounds, for example, di- and tri-nitrotoluene, or nitric acid esters of polyhydroxy compounds such as nitroglycerin, nitroglycol, nitromannite, and pentaerythritol tetranitrate, or other explosive organic nitrates or nitro compounds, for example, nitramines such as nitroguanidine. Other agents may be included for securing desired characteristics such as, for example, stabilizers, deterrents, waterproofing agents, and other substances adapted to produce specific effects.

Although the smokeless powder base employed may be one which has been brought to a condition of stability by previous treatments, the procedure of this invention is likewise well adapted for converting an incompletely purified and unstable starting material to a product having satisfactory stability. The rate of the purification and stabilization reactions is enhanced by the elevated pressure which makes possible the utilization of elevated temperature in the treatment and the increase in fluidity of the lacquer as a consequence.

When nitrocellulose is utilized as the smokeless powder base, it may be used in the fibrous state, either after having been stabilized by suitable treatments or as freshly nitrated cellulose which has merely been washed to remove occluded acid. The starting material may likewise consist of previously colloided nitrocellulose which may have become deteriorated by the effect of long storage even to such an extent as to contain decomposed spots of relatively high acidity. Similarly, the raw material may consist of colloided nitrocellulose-nitroglycerin powders.

The medium in which the steps of grain formation and subsequent removal of solvent occur is one which is not a solvent for the smokeless powder base. Water constitutes the medium which is preferred as a general rule and from the economical standpoint for such use. It will be understood, however, that other nonsolvent liquids may at times be useful, for example, solvent naphtha or chlorinated hydrocarbons such as carbon tetrachloride, provided always that the

non-solvent selected be one which is not substantially miscible with the solvent selected.

The solvent used to disperse the smokeless powder base in lacquer form is one which is substantially immiscible with the non-solvent medium above referred to and which is sufficiently volatile as to be readily removed from the lacquer by evaporation. Generally, the solvent should have a boiling point below or not greatly in excess of 100° C. although solvents of somewhat higher boiling points may at times be suitable. When water is employed as the non-solvent medium and nitrocellulose as the smokeless powder base, esters such as ethyl acetate, isopropyl acetate, butyl acetate, or ethyl formate, or water-immiscible ketones such as methyl ethyl ketone or methyl isobutyl ketone may be employed. However, with the use of a non-solvent medium other than water, solvents such as acetone or ether-alcohol may be used, provided they are not substantially miscible with the non-solvent medium selected.

The amount of solvent most suitable for use in any given instance will depend largely on the particular smokeless powder base employed and the temperature of the graining operation. For example, in a case where pyronitrocellulose containing about 12.5% nitrogen is formed into spherical grains at a temperature of 70°-85° C., an amount of ethyl acetate equal to 1½-4 times the weight of powder base may be employed. As a general rule, the lower the viscosity of the nitrocellulose, the lower the proportion of solvent need be. For example, with a wood nitrocellulose having a viscosity of about 17 seconds (Hercules method) advantageous results are accomplished when the amount of ethyl acetate employed is 3.65 times the weight of the nitrocellulose, whereas with nitrocellulose having a viscosity of about 5 seconds, the proportion of ethyl acetate to nitrocellulose may be reduced to 3-to-1.

In order to form the desired globules of the smokeless powder base lacquer, the smokeless powder base, a limited quantity of solvent therefor, and water or other suitable non-solvent medium, sufficient in amount to permit adequate agitation of the mixture, and preferably having a protective colloid dispersed therein, are mixed at a sufficiently elevated temperature that a fluid and mobile smokeless powder base lacquer results, but in order to inhibit loss of solvent from the lacquer at such elevated temperatures the pressure upon the mixture is increased substantially above atmospheric. The agitation is sufficient to distribute the lacquer into particles of desired size and is carried out under conditions such that evaporation of solvent does not occur. After agitation for a sufficient period, the particles assume a spherical shape probably largely due to the effect of interfacial tension forces. When this stage has been reached, the pressure on the mixture is reduced either by venting to the atmosphere or by rapidly cooling the mixture, which results in setting the globules of lacquer in their acquired spherical shape, in the one case by reducing the influence of heat and in the other case by reducing the influence of solvent toward fluidity of the lacquer. After the globules are thus set and while still maintained in suspension, additional heat may be supplied to remove solvent from the globules by distillation. In order to effect substantially complete removal of solvent the temperature may be gradually increased during the distillation peri-

od, the pressure upon the mixture during this final distillation stage being preferably at or about atmospheric.

It will be understood that other desired ingredients may be present during the graining operation. Where the smokeless powder base consists of deteriorated or unpurified nitrocellulose, the treatment is preferably carried out in the presence of a mild alkaline material, such as calcium carbonate, sufficient to neutralize the excess acidity present in the starting material. Furthermore, the desired amount of stabilizers such as diphenylamine, or a dialkyldiphenylurea such as methyl centralite, deterrents such as dinitrotoluene or dibutyl phthalate, accelerators such as nitroglycerin, or waterproofing agents may be present in the mixture. Protective colloids such as starch, gum arabic, dextrin, animal glue or bentonite may be utilized to facilitate and control the granulation process, as disclosed in the said U. S. Patent 2,027,114. In order to control the density of the product, solutes may be utilized as disclosed in U. S. Patent 2,160,626.

The process may be controlled so that grains of predetermined size and density are produced by suitable adjustment of various factors, as disclosed in the aforesaid U. S. Patent 2,027,114. Thus the average grain size may be decreased by increasing the violence of the agitation or by increasing the amount of protective colloid present, or by decreasing the viscosity of the smokeless powder base lacquer, as by the use of more solvent or by raising the temperature of the graining operation. The average grain size may be increased by changing these variables in the opposite direction.

In order to illustrate the process of this invention, a detailed description is given below of the practice followed in manufacturing smooth-surfaced spherical grains of smokeless powder with the use of finely divided nitrocellulose as starting material. This raw material may be obtained, for example, by grinding granular colloided nitrocellulose in the presence of water and screening the resulting powder through a suitable screen, for example, one finer than 8 mesh.

The steps of forming the grains and removing the volatile solvents may conveniently be carried out in a single vessel provided with the necessary facilities, such as means for heating and cooling the contents, for example a suitable jacket through which cooling or heating fluid may be circulated; suitable means for agitation, such as a rotatable shaft on which are mounted a plurality of horizontally disposed blades, the action of which may be supplemented by baffles which project inwardly from the sides of the vessel; an orifice at the top for charging the vessel and a cover for sealing the same; an outlet at the bottom of the vessel for discharging the contents and a suitable valve for opening and closing the same; and a vapor outlet leading to a condenser, furnished with a valve which may be opened or closed at will.

Four hundred pounds of finely divided colloided nitrocellulose in the form of a mud in which the individual particles are finer than 60 mesh, 4800 pounds of water, and 4 pounds of finely divided calcium carbonate were added to a vessel of the above type. This mixture was violently agitated by rotating the agitator at a sufficient rate so that the contents were in a turbulent state and the surface broken up into a number of vortices. While maintaining the agitation, the temperature of the mixture was raised to 50° C. by cir-

culating hot water through the jacket. Twelve hundred pounds of ethyl acetate containing 8 pounds of dinitrotoluene and 1 pound of diphenylamine in solution were then added over a period of about 45 minutes while the violent agitation was maintained and the temperature was being raised to 55° C. The vapor outlet of the vessel was then closed and the contents were heated rapidly to 75° C., the pressure rising to 12.5 pounds per square inch above atmospheric.

At this point the agitation was stopped and the mixture was allowed to separate into two layers, a bottom aqueous layer, and an upper layer of nitrocellulose-ethyl acetate lacquer containing droplets of water emulsified therein. During the stationary separation period of about 15 minutes, a solution of 14 pounds of gum arabic in 50 pounds of hot water was added to the vessel from a pressure tank maintained at about 25 pounds per square inch pressure above atmospheric.

Violent agitation was then resumed and continued for a brief period, for example, about 4 or 5 minutes. This resulted in the separation of the lacquer into irregularly shaped particles, each of which was subsequently to be transformed into a spherical grain of smokeless powder. In order to accomplish this transformation of irregular particles to globules, the mixture was maintained for a period of 2 hours at about 75° C. during agitation sufficient to maintain the globules in suspension in the freely swirling liquid while keeping the surface of the liquid smooth and unbroken.

During the grain shaping period, the density of the resulting powder grains may be controlled in accordance with the process disclosed and claimed in U. S. Patent 2,160,626. For example, in order to increase the density of the product produced in accordance with the present example, a solution containing 75 pounds of sodium sulfate (calculated on the basis of anhydrous salt) in 400 pounds of water was added under pressure during the first 15 minutes of the grain shaping period.

When the grains had assumed globular form, the temperature of the suspension was reduced to 60° C. and the excess pressure above atmospheric was relieved by opening the vapor line leading to the condenser. At this temperature, the lacquer globules became "frozen" in their acquired form due principally to the greatly increased viscosity of the lacquer.

The solvent was then removed from the globules by a distillation process in which the temperature was gradually increased, for example, according to a schedule in which the temperature was raised to 65° C. in 45 minutes, then maintained during successive one hour periods at 65°-70° C., at 70°-75° C., and then at 75°-87° C., and finally for 90 minutes at 87°-94° C. The water and solvent vapor evolved from the suspension were caused to pass at atmospheric pressure through a condenser, the recovered solvent being suitable for reuse in the process.

After removal of the solvent as above described, the suspension was cooled to room temperature, the powder grains were recovered by filtration or by means of a centrifuge and washed with warm water in order to remove the protective colloid and salt. The grains could then be subjected to a screening operation for separating the over-sized and under-sized grains from the product. The globular grains of gelatinized nitrocellulose resulting from this procedure had a gravimetric density of 0.837 and a majority

of the grains were between .012-0.24 inch in diameter.

The powder grains at this stage may be subjected to any further desired processing step, for example, to a surface treatment with a modifying agent such as an accelerator and/or a detergent. After drying and graphiting, the powder grains may be stored ready for use.

When a final product having different characteristics is desired, the manufacturing procedure may be varied from the above in order to secure greatest economy of operation. For example, in the production of spherical grains having an average diameter of 0.01 inch, more rapid agitation may be employed and a grain shaping period of 30 minutes followed by a distillation period of 3-4 hours yield excellent results.

The relatively high fluidity of the lacquer of the smokeless powder base at the elevated temperature of the graining step causes the transformation of the dispersed particles of lacquer into globular shape to occur quite readily, while the increased viscosity of the lacquer at the lower temperature provided after the graining step imparts to the globules a marked resistance to deformation during the unavoidable collisions with other globules, with the agitating means, and with the walls of the vessel incident to agitation during the step of removing the solvent.

As illustrating a further embodiment of the invention wherein reduction of pressure upon the mixture after the globules have been formed is accomplished without chilling but by venting the sealed vessel containing the mixture, 3300 pounds of fibrous wood nitrocellulose (containing 13.4% nitrogen) and 41 pounds of finely divided chalk are suspended in 26,000 pounds of water and the resulting suspension, after being heated to a temperature of 50°-55° C., is pumped into the distillation vessel. 10,400 pounds of ethyl acetate, containing 33 pounds diphenylamine, are then added to the suspension during agitation. The suspension is then heated to a temperature of 80° C. in about 45 minutes, the vessel being sealed so that a pressure of about 15 to 20 pounds per square inch above atmospheric is developed, depending upon the amount of air which is present.

The agitation is discontinued for a period of about 15 minutes, permitting the nitrocellulose solution to coalesce as a separate layer above the water. During this time, a protective colloid solution is added, for example a solution of 120 pounds of a good grade animal bone glue in 1500 pounds of water.

Agitation is then resumed, and 15 minutes later a solution of 475 pounds of sodium sulfate in 1500 pounds of water is added. After a total of about 2 hours agitation at 80° C., the graining and shaping of globules is completed.

While the temperature is maintained at 80° C., the outlet valve to the condenser is gradually opened until a decrease in pressure is noted on the pressure gauge. The pressure decreases to about 5 pounds per square inch gauge in about 10 to 15 minutes, venting of air accounting for most of this pressure drop. The distillation of solvent starts at this point and continues for a period of about 60 minutes, the pressure in the distillation vessel being reduced gradually to atmospheric by further opening the outlet valve to the condenser at intervals. About 80% of the solvent is removed during this time.

While the above described gradual decrease of pressure can be accomplished by careful

manual operation of the outlet valve, it is generally preferable to provide automatic pressure release according to a predetermined schedule.

The temperature of the suspension is then raised to about 95° C. in 45 minutes and maintained at this point for about 15 minutes to complete the solvent removal treatment. After cooling, the charge may be centrifuged, washed, and screened and subjected to any other finishing treatment that may be desired.

The product of the foregoing process consists of globular grains of gelatinized nitrocellulose, displaying a gravimetric density of .930 and of which about 74% have a diameter between 0.010 and 0.025 inch, 14% being smaller than 0.010 inch in diameter and 12% being larger than 0.025 inch in diameter.

In the manufacture of globular smokeless powder grains, in accordance with the present invention economy is secured not only by virtue of the reduction in the amount of solvent required but also because a shorter period is required for forming the grains and for removing the solvent. Likewise, the rate of solvent removal may be much higher than for globules which contain a much higher proportion of solvent, since due to the reduced shrinkage obtained on removing solvent from globules which initially contain a high solids content, there is less danger of deforming the grains by shrinkage thereof. The process of this invention, due to the latter factor, is particularly suited for the production of dense grains.

It will be understood that an important aspect of my improved process is the carrying out of the step of graining, or globule formation, at pressures substantially above atmospheric which makes it possible to utilize temperatures sufficiently high that the heat contributes toward increasing the fluidity of the lacquer, without, however, depleting the lacquer of solvent. The graining step is followed by lowering of the pressure, which may or may not be attended by a lowering in temperature, in order to set the grains in their acquired form, and finally, the residual volatile solvent may be substantially removed, as by evaporation. The operating details hereinbefore described are to be considered as illustrative of the invention and not limitative, and many variations may be made within its spirit and scope as will be realized by those skilled in the art when the present description is read. Such variations may include, for example, the utilization of other smokeless powder bases, other solvents, and other suspension media, as hereinbefore described, as well as changes in the temperatures, concentrations, and times of treatment which are subject to adjustment to give the most desirable results in each particular instance.

Having now described the invention, what is claimed as new and is desired to be secured by Letters Patent, is:

1. In the art of making explosives, the process comprising, agitating nitrocellulose and 1½ to 4 times its weight of a water-immiscible solvent therefor in an aqueous bath, heating the mixture to 70°-85° C. during agitation without removal of solvent to form a suspension of fluid particles of nitrocellulose solution, continuing the agitation under the said conditions to form the said particles into globular shape, and cooling the suspension to about 60° C. to rigidify the said globules.

2. In the art of making explosives, the process comprising, suspending particles of smokeless

powder base solution in a non-solvent liquid at an elevated temperature sufficiently high to render the solution fluid, said non-solvent liquid being substantially immiscible with the solution agitating the suspension while avoiding the removal of solvent from the solution to form globules thereof, then cooling the suspension to rigidify the said globules, and thereafter removing solvent.

3. In the art of making explosives, the process comprising, agitating a smokeless powder base in a non-solvent liquid with solvent which is immiscible with and has a lower boiling point than the liquid, the solvent being sufficient in amount to render the said base fluid at a temperature above the normal boiling point of the mixture, heating the mixture in a sealed vessel to the said temperature, continuing the agitation under the said conditions to form globules of smokeless powder base solution, and then cooling the suspension below the boiling point of the mixture to rigidify the said globules.

4. In the art of making explosives, the process comprising, agitating a smokeless powder base in a non-solvent liquid, adding solvent substantially immiscible with the liquid in an amount insufficient to render the said base fluid at the temperature of admixture but sufficient therefor at a higher temperature, heating the mixture to the said higher temperature while concurrently comporting the temperature and pressure of the mixture with the vapor pressure of the solvent to substantially avoid removal of solvent from the solution, continuing the agitation under the said conditions to form globules of the solution, and then cooling the suspension to rigidify the said globules.

5. In the art of making explosives, the process comprising, agitating a smokeless powder base in a non-solvent liquid with solvent which is immiscible with and has a lower boiling point than the liquid, the solvent being insufficient in amount to render the said base fluid at below the boiling point of the mixture but sufficient therefor at a higher temperature, heating the mixture in a sealed vessel, to above the normal boiling point of the mixture, continuing the agitation under the said conditions to form globules of smokeless powder base solution, and then cooling the suspension below the boiling point of the mixture to rigidify the said globules.

6. In the art of making explosives, the process comprising, agitating a smokeless powder base in a non-solvent liquid with solvent which is immiscible with and has a lower boiling point than the liquid, the solvent being sufficient in amount to render the said base fluid at a temperature above the boiling point of the mixture, heating the mixture in a sealed vessel to the said temperature and to a pressure above atmospheric, continuing the agitation under the said conditions to form globules of smokeless powder base solution, and thereafter removing solvent at atmospheric pressure.

7. The process of claim 2, in which the smokeless powder base consists of nitrocellulose.

8. The process of claim 2, in which the smokeless powder base consists of nitrocellulose-nitro-glycerin.

9. The process of claim 2, in which the smokeless powder base consists of nitrostarch.

10. In the art of making explosives, the process comprising, agitating nitrocellulose and about three times its weight of a water-immiscible solvent in an aqueous bath, heating the mixture to substantially 75° C. during agitation to form a

suspension of fluid particles of nitrocellulose solution, continuing the agitation under the said conditions to form globules of the solution, concurrently with said heating and agitation comporting the temperature and pressure of the mixture with the vapor pressure of the solvent to substantially avoid removal of solvent and cooling the suspension to about 60° C. to rigidify the said globules.

10 11. In the art of making explosives, the process comprising, agitating a smokeless powder base in a non-solvent liquid with solvent which is immiscible with the liquid, the solvent being insufficient in amount to render the said base fluid at an intermediate temperature above atmospheric but sufficient therefor at a higher temperature, heating the mixture to the said higher temperature, continuing the agitation under the said conditions to form globules of the solution, concurrently with said heating and agitation comporting the temperature and pressure of the mixture with the vapor pressure of the solvent to substantially avoid removal of solvent and then cooling the suspension to the said intermediate temperature to rigidify the said globules.

12. In the art of making explosives, the process comprising, agitating a solution of smokeless powder base in a non-solvent liquid, the solvent for said solution being immiscible with the liquid, the solvent being sufficient in amount to render the said base fluid at a temperature above the normal boiling point of the mixture, heating the mixture in a sealed vessel with concomitant increase in pressure to a temperature above the normal boiling point of the mixture, continuing the agitation under said conditions to form globules of smokeless powder base solution, then reducing the pressure in the vessel while agitation continues.

40 13. In the art of making explosives, the process comprising, agitating a solution of smokeless powder base in a non-solvent liquid, the solvent for said solution being immiscible with and having a lower boiling point than the liquid, the solvent being sufficient in amount to render the said base fluid at a temperature above the atmospheric pressure boiling point of the mixture, heating the mixture in a sealed vessel with concomitant increase in pressure to a temperature above the boiling point of the mixture at atmospheric pressure, continuing the agitation under said conditions to form globules of smokeless powder base solution, then reducing the pressure in the vessel while agitation continues, and thereafter under reduced pressure distilling solvent from the mixture.

14. In the art of making explosives, the process comprising, agitating a solution of smokeless powder base in a non-solvent liquid, the solvent for said solution being immiscible with and having a lower boiling point than the liquid, the solvent being sufficient in amount to render the said base fluid at a temperature above the atmospheric pressure boiling point of the mixture, heating the mixture in a sealed vessel with concomitant increase in pressure to a temperature above the boiling point of the mixture at atmospheric pressure, continuing the agitation under said conditions to form globules of smokeless powder base solution, then reducing the pressure in the vessel while agitation continues, and thereafter under pressure about atmospheric distilling solvent from the mixture.

15. In the art of making explosives, the process comprising, agitating a smokeless powder base in

a non-solvent liquid with solvent which is immiscible with and has a lower boiling point than the liquid, the solvent being sufficient in amount to render the said base fluid at a temperature above the boiling point of the mixture, but insufficient in amount to render said base fluid at atmospheric temperatures, heating the mixture under pressure above atmospheric to a temperature above the atmospheric pressure boiling point of the mixture, continuing the agitation under the said conditions to form globules of smokeless powder base solution, and thereafter, under reduced pressure, distilling solvent from the mixture.

16. In the art of making explosives, the process comprising, agitating nitrocellulose base powder in a bath of water with ethyl acetate, there being approximately 3 to 4 parts, by weight, of ethyl acetate to each part of base powder, concurrently agitating and heating the mixture in a sealed vessel to a temperature of about 80° C. with concomitant increase in pressure to about 15 to 20 pounds per square inch above atmospheric pressure, without reducing the temperature and pressure discontinuing the agita- 25

tion for a time sufficient to permit the base powder solution to coalesce, resuming the agitation and continuing the same until the smokeless powder base solution is dispersed as globules in the water, all without reducing the temperature or pressure upon the mixture, then gradually reducing the pressure within the vessel to between zero and 5 pounds per square inch above atmospheric while maintaining the temperature, and continuing the heating at such reduced pressure until the ethyl acetate is substantially removed from the globules.

17. In the art of making explosives, the process comprising, suspending particles of smokeless powder base solution in a non-solvent liquid at an elevated temperature above the normal boiling point of the mixture to render the solution fluid, said non-solvent liquid being substantially immiscible with the solution agitating the suspension under pressure while avoiding the removal of solvent from the solution to form globules thereof, then reducing the pressure while agitation continues.

CHARLES EARNEST SILK.